

## UNITED STATES PATENT OFFICE

HENRI LOUIS BARTHELEMY, OF MILAN, ITALY, ASSIGNOR TO RUTHALDO COMPANY INC., OF NEW YORK, N. Y., A CORPORATION OF NEW YORK

MANUFACTURE OF THREADS, RIBBONS, FILMS, AND THE LIKE FROM SOLUTIONS OF CELLULOSE ESTERS AND CELLULOSE ETHERS

No Drawing. Application filed July 28, 1927, Serial No. 209,163, and in France December 28, 1926.

This invention relates to the manufacture of artificial silk filaments, bands, films and the like, from solutions of cellulose esters or cellulose ethers.

5 It consists in forcing a solution obtained in known manner (for instance, by dissolving cellulose acetate, cellulose formate, cellulose nitrate or mixed esters) through a nozzle sprayed with or immersed in a special coagulating or precipitating liquid hereinafter described; or more simply in distributing said solution in the form of filaments or thin bands on means (such as a flat surface, an endless band or a drum with a dull or polished surface) which is sprayed with, or 10 immersed in, said coagulating or precipitating liquid.

Said liquid may consist of an aqueous solution of ammonium oleate, potassium oleate 20 or sodium oleate, and these substances may be used either separately or mixed together; or it may consist, in general, of any aqueous solution which contains an ammonium or alkali salt of one or more fatty acids (which 25 may even be sulfonated), for instance, ammonium stearate, potassium palmitate or sodium ricinoleate, sulfopalmitates or sulfoncinoleates of ammonium or sodium etc.

It has also been found that by the addition 30 of members of a group of compounds adapted to form aqueous emulsions in the bath, still better results may be obtained, for instance, in regard to the elasticity and lustre of the final product.

35 These compounds may be divided into four groups:

(1) Simple alcohols and polyhydric alcohols; such as ordinary alcohol, butyl alcohol, glycol, glycerol, and cyclohexanol, which 40 may be employed separately or mixed together.

(2) Hydrocarbons; such as decane, tridecane, hexadecane, toluene, the three xylenes, tetralin, decalin, terpenes, sesquiterpenes, 45 polypropenes, mineral oils and so on.

(3) Fatty acids of high molecular weight and their alkyl esters; such as methyl oleate, ethyl oleate, methyl stearate, and so on.

(4) The animal and vegetable oils which 50 not only emulsify readily, but also with

proper concentration of the emulsifying agent, furnish what appear to the eye to be homogeneous mixtures with water.

It should be noted that the invention differs substantially from certain known processes which aim at carrying out the spinning process in a single compound, for instance in oil of turpentine or in animal or vegetable oils.

The present invention presents a great advantage over known processes, inasmuch as when mineral or vegetable oils are added, the prior emulsification of the fatty substances enables the filaments or films to be cleaned in a very simple manner by merely washing 60 in lukewarm water, as a result of the known cleansing action of alkaline soaps, the sulfonates sulfopalmitates and the like.

Furthermore, on coagulation, the threads are thoroughly lubricated by the coagulant 70 solution itself, since the latter acts in the same manner as a true lubricating oil owing to the simultaneous presence of a fatty oil with a sulforicinoleate or an alkaline soap. This fact enables the filaments to be subjected to mechanical treatment with far 75 great ease than is possible in the ordinary spinning process for producing artificial silk.

The presence of a soluble salt of a fatty acid or sulfonated fatty acid offers the further advantage of considerably reducing surface tension, thereby on the one hand accelerating the diffusion of the solvent in the bath and on the other hand reducing the mutual adhesion of the filaments in the production of 85 artificial silk.

Instead of emulsifying agents specified above one may use caseinates, gums, soaps, alkaline salts, etc., or mixtures thereof.

In fact I may use as an emulsifying agent 90 any substance which, when mixed with water, will diminish the surface tension of the water. Soaps and oils are particularly beneficial, as they both act as colloids but more especially they diminish the surface tension of the 95 water.

The apparatus in which the precipitation is effected may be so designed that the solvent for the cellulose esters can be continuously recovered by simple distillation, so that the 100

drained and cooled bath may be used over and over again for precipitating fresh quantities of films or threads, on issuing from the dephlegmator.

5 *Example*

48 parts of a 50% solution of ammonium oleate are mixed with 40 parts of neat's-foot oil and 12 parts of mineral oil. A 19.8% 10 solution of cellulose acetate in acetone is forced into this emulsion under a pressure of 3 kg. per sq. cm., through a silver spinning nozzle of 0.32 mm. bore. After washing the thread in lukewarm water an elastic silk yarn 15 of excellent lustre is obtained.

Having now fully described my invention, what I claim and desire to secure by Letters Patent is:—

1. A process of manufacturing artificial 20 threads, films, ribbons and the like, which consists in forcing a solution of cellulose acetate in acetone into an aqueous emulsion containing a solution of ammonium oleate mixed with neat's-foot oil and mineral oil.

2. A process of manufacturing artificial 25 threads, films, ribbons and the like, which consists in forcing an approximately 19.8% solution of cellulose acetate in acetone into an aqueous emulsion containing about 48 parts 30 of a 50% solution of ammonium oleate, 40 parts neat's-foot oil and 12 parts of mineral oil.

3. A process of manufacturing artificial 35 threads, films, ribbons and the like, which consists in introducing acetone solutions of cellulose esters into an emulsified aqueous bath containing a slightly soluble organic liquid and an emulsifying agent.

4. A process of manufacturing artificial 40 threads, films, ribbons and the like, which consists in introducing a solution of cellulose acetate in acetone into an aqueous bath comprising an oil emulsified in an aqueous solution of ammonium oleate.

45 5. A process of manufacturing artificial threads, films, ribbons and the like, which consists in introducing acetone solutions of cellulose esters into a mixture of an emulsifying agent in water and an emulsified compound dispersed in the mixture.

60 6. A process of manufacturing artificial threads, films, ribbons and the like, which consists in precipitating or forcing acetone solutions of cellulose esters into an aqueous 55 coagulating bath composed of an emulsifying agent in water and an emulsified compound dispersed in the mixture, said compound being a solvent of the solvent employed for the preparation of the cellulose acetate 65 solution.

65 7. A process of manufacturing artificial threads, films, ribbons and the like, which consists in precipitating or forcing acetone 70 solutions of cellulose esters into an emulsified mixture of water and compounds which are

not solvents of esters of cellulose, and which compounds added to water will diminish its surface tension.

8. A process of manufacturing artificial 75 threads, films, ribbons and the like, which consists in precipitating or forcing acetone solutions of cellulose esters into an aqueous mixture containing oil and an emulsifying agent.

9. A process of manufacturing artificial 75 threads, films, ribbons and the like, which consists in coagulating cellulosic ester solutions in a mixture of water and a material giving an emulsion with water.

10. A process of manufacturing artificial 80 threads, films, ribbons and the like, consisting in coagulating solutions of cellulose esters in an aqueous mixture composed of water, and an organic compound insoluble in water and a chemical compound which emulsifies 85 the organic compound in the water.

11. A process of manufacturing artificial 90 threads, films, ribbons and the like, consisting in coagulating solutions of cellulose esters in a mixture of water, a material having the 95 property of lowering the surface tension of water and of emulsifying fatty substances, and an organic solvent of the cellulose ester to be spun.

12. The manufacture of cellulosic products 95 consisting in entering a solution of a cellulose ester in filament form into a coagulating bath consisting of an aqueous emulsion of oil.

13. The manufacture of cellulosic products 100 consisting in entering a solution of a cellulose ester in filament form into a coagulating bath consisting of water and oil emulsified by means of a soap.

14. A process of manufacturing artificial 105 threads, films, ribbons and the like, which consists in precipitating an acetone solution of a cellulose ester in an emulsified aqueous liquid mass containing acetone.

15. A process of manufacturing artificial 110 threads, films, ribbons and the like, which consists in precipitating acetone solutions of cellulose esters in an emulsion of water and liquids which are not solvents of the cellulose ester used.

In testimony whereof I affix my signature. 115  
HENRI LOUIS BARTHELEMY.

120

125

130